

Jan. 5, 1932.

K. L. SCOTT

1,839,344

METHOD OF TREATING MAGNETIC MATERIALS

Filed Nov. 8, 1927



Fig. 1.



Fig. 2.



Fig. 3.

Inventor  
Kenneth L. Scott  
by Malikian Atty.

## UNITED STATES PATENT OFFICE

KENNETH LOYAL SCOTT, OF WESTERN SPRINGS, ILLINOIS, ASSIGNOR TO WESTERN ELECTRIC COMPANY, INCORPORATED, OF NEW YORK, N. Y., A CORPORATION OF NEW YORK

## METHOD OF TREATING MAGNETIC MATERIALS

Application filed November 8, 1927. Serial No. 231,934.

This invention relates to a method of treating magnetic materials, and more particularly to a method of heat treating magnet steel.

6. An object of the invention is to provide a method for improving the magnetic properties of magnet steel.

In accordance with the general features of the invention, the magnet steel, such as cobalt or tungsten steel is first brought to approximately its maximum magnetic hardness at which point it would, after being magnetized to saturation, have a certain residual induction. The steel is then tempered to an intermediate degree of hardness which cannot be obtained directly, after which it will, after being magnetized to saturation, have an increased residual induction. By magnetic hardness is meant that quality of a magnetic material which causes it to resist magnetization and demagnetization. In a given material, it is proportional to the coercive force but is not proportional to the residual induction as will appear more fully below.

25. It is believed that a complete understanding of the invention may be had by reference to the following description taken in conjunction with the accompanying drawings, in which

30. Fig. 1 is a graphic representation of phenomena encountered in the hardening of cobalt steel;

Fig. 2 represents hysteresis loops of cobalt steel showing its magnetic properties in the hardened and tempered states, and

35. Fig. 3 is a graphic representation of the properties of cobalt steel upon hardening and tempering.

The invention will be described in connection with cobalt steel although other steels such as tungsten steel respond to the same method of treatment. The hardening of cobalt steel is accomplished by heating the steel to a temperature of about 1700° F. or slightly above the  $A_2$  transformation point and then quenching the steel in oil, water or other suitable quenching medium. It has been found that in heat treating the cobalt steel by raising its temperature to a certain value and then quenching there is no marked increase in the

magnetic hardness of the steel until the temperature is brought to a value between 1600° F. and 1700° F., which is above the  $A_2$  transformation point before quenching. This is shown graphically in Fig. 1 in which the abscissas represent the temperature in degrees Fahrenheit to which a specimen has been raised before quenching, and the ordinates represent the magnetic coercive force in gilberts per centimeter necessary to bring a specimen which has been magnetized to saturation back to zero magnetization. Since the coercive force varies with magnetic hardness, the curve in Fig. 1 may be taken to represent the variations in magnetic hardness in specimens of steel which are raised to the different values of temperature shown by the abscissas and then quenched.

It will be noted that the curve in Fig. 1 is practically vertical for a considerable distance indicating that different degrees of magnetic hardness may be obtained at a single temperature value. The particular magnetic hardness obtained at this temperature is theoretically indeterminate and may be ascertained only by test.

In experimenting with the heat treatment of cobalt steel it was discovered that if a specimen of the steel is first brought to its maximum magnetic hardness, its residual induction after magnetization to saturation may be greatly increased by subsequently tempering it to a lower magnetic hardness, in which tempering process any desired degree of magnetic hardness may be obtained by reheating the steel to an appropriate temperature.

The improvement in the residual induction of a specimen of cobalt steel upon tempering it to a lower degree of magnetic hardness after hardening to its maximum extent is shown graphically in Fig. 2 in which the abscissas indicate magnetizing forces in gilberts per centimeter and the ordinates indicate flux densities in maxwells per square centimeter. The curve 5 represents a hysteresis loop of a specimen of cobalt steel brought to its maximum hardness and the curve 6 represents a hysteresis loop of a tempered specimen. It will be noted that the 100

residual induction of the tempered specimen, indicated by the point where the loop 6 intersects the vertical axis, is considerably higher than the residual induction of the specimen at its maximum hardness, indicated by the point where the loop 5 intersects the vertical axis. Incidentally it may be observed that while the magnetizing force necessary to reduce the flux density to zero after the specimens have been magnetized is less in the tempered specimen than in the specimen which was brought to its maximum hardness, as long as the coercive force is not reduced below a certain limiting value, which will depend upon the dimensions of the magnets to be made from the steel, this fact is of little consequence.

In Fig. 3, in which the abscissas indicate magnetizing forces in gilberts per centimeter and the ordinates indicate remanence in maxwells per square centimeter, the curve 7 represents the magnetic remanence of permanent magnets, such as bars or horseshoes, brought to various degrees of magnetic hardness and the curve 8 represents the magnetic remanence of similar magnets tempered to various degrees of hardness from their maximum values, showing a maximum magnetic remanence at an intermediate degree of magnetic hardness of the metal between maximum hardness and minimum hardness in the tempered specimen.

In a specific application of the method of improving the magnetic properties of steel, a magnet containing approximately 36% of cobalt is heated to a temperature of 1700° F. and quenched in oil or water, bringing it to substantially its maximum hardness. The magnet is then reheated to a temperature not to exceed 1300° F. and quenched in air tempering it to a lesser degree of magnetic hardness, increasing the residual induction of the material, and thereby increasing the magnetic remanence of the magnet.

It will be understood that the embodiment of the invention herein described and illustrated is merely a convenient and useful form of the invention which is capable of many other modifications without departing from the spirit and scope of the invention.

What is claimed is:

1. A method of improving the magnetic properties of magnet steel containing 5% to 60% cobalt, which comprises heating the steel to a temperature adapted to produce a high degree of magnetic hardening, quenching the steel, reheating to a lower temperature adapted to produce an intermediate degree of magnetic hardening, and quenching the steel.

2. A method of improving the magnetic properties of steel containing 5% to 60% cobalt, which comprises heating the steel to a temperature of approximately 1700° F., quenching the steel, reheating the steel to a

temperature not to exceed 1300° F., and quenching the steel.

3. A method of improving the magnetic properties of steel containing 5% to 60% cobalt, which comprises heating the steel to a temperature adapted to produce a high degree of magnetic hardening, quenching the steel rapidly, reheating to a lower temperature adapted to produce an intermediate degree of magnetic hardening, and quenching the steel slowly.

4. The method of improving the magnetic properties of cobalt magnet steel, which comprises rapidly quenching the steel from a temperature of approximately 1700° F. to produce a high degree of magnetic hardening, and subsequently quenching the steel from a temperature not exceeding 1300° F. to produce an intermediate degree of magnetic hardening.

5. A method of improving the magnetic properties of cobalt magnet steel, which comprises heating the steel to a temperature adapted to produce a high degree of magnetic hardening, quenching the steel, reheating the steel to a temperature adapted to produce an intermediate degree of magnetic hardening, and slowly cooling the steel.

6. The method of improving the magnetic properties of cobalt magnet steel, which comprises heating and quenching the steel to bring it substantially to its maximum magnetic hardness, and subsequently reheating and slowly cooling the steel to produce a lesser degree of magnetic hardness whereby its magnetic remanence is increased.

7. The method of improving the magnetic properties of steel containing 36% cobalt, which comprises rapidly quenching the steel from a temperature of approximately 1700° F. to produce a high degree of magnetic hardening, and subsequently quenching the steel from a temperature not exceeding 1300° F. to produce an intermediate degree of magnetic hardening.

8. A method of improving the magnetic properties of steel containing 36% cobalt, which comprises heating the steel to a temperature adapted to produce a high degree of magnetic hardening, quenching the steel, reheating the steel to a temperature adapted to produce an intermediate degree of magnetic hardening, and slowly cooling the steel.

9. The method of improving the magnetic properties of magnet steel containing 36% cobalt, which comprises heating and quenching the steel to bring it substantially to its maximum magnetic hardness, and subsequently reheating and slowly cooling the steel to produce a lesser degree of magnetic hardness whereby its magnetic remanence is increased.

10. The method of improving the magnetic properties of cobalt steel, which comprises heating the steel to a temperature above its  $A_2$  transformation point, then quickly cool-

ing the steel, then reheating the steel to a temperature adapted to produce an intermediate degree of magnetic hardening but not above 1300° F., and then cooling the steel.

5 In witness whereof, I hereunto subscribe my name this 25th day of October A. D., 1927.

KENNETH LOYAL SCOTT.

10

15

20

25

30

35

40

45

50

55

60

65